

## UNITED STATES PATENT OFFICE

2,607,742

## METALLIC GETTER COMPOSITIONS

Lloyd D. Lockwood, Millburn Township, Essex County, N. J., assignor to Tung-Sol Lamp Works, Inc., Newark, N. J., a corporation of Delaware

No Drawing. Application December 30, 1949,  
Serial No. 136,138

12 Claims. (Cl. 252—181.2)

1

This invention relates to getter compositions embodying metallic getter powders and binders therefor.

One object of the invention is a novel and improved getter paint.

A further object of the invention is a novel and improved binder for metallic getter powders.

A further object of the invention is a novel and improved binder for metallic getter powders which also acts as a getter.

A further object of the invention is a novel method of making a paint of the above indicated character.

Further objects of the invention will hereinafter appear.

In the conventional practice of manufacturing electric incandescent lamps, vacuum tubes and the like with which I am familiar, the fine metal getter powders that are painted or sprayed on metal plates or lead wires are retained by some carbon compound as a binder. For example, binders of nitro cellulose, cellulose acetate, shellac, and sugar compounds have been proposed and also one made from ethyl silicates. All of these binding materials eventually release carbon which if taken out of the lamp or envelope in the gas form does no damage but if carbon is left behind in the lamp envelope it tends to form or forms tungsten carbide. Tungsten carbide is very brittle and having a different coefficient of expansion from that of tungsten, of which the filament is made, causes the tungsten to distort or become distorted. This in turn results in broken filaments and unduly short life.

Regardless of how good or effective the metallic getter powder is, the results in lamps have not been satisfactory and I have found that this is due to the effect of the presence of carbon released from the binders. I have found that a satisfactory lamp getter must take care of, or get out of the lamp three things instead of the two we usually consider. They are hydrogen, oxygen and carbon.

A number of metallic powders make good getters and of these zirconium is probably the best and most satisfactory. It is capable of taking up hydrogen, oxygen and carbon at the temperatures found on miniature lamp lead wires as, for example, lead wires of nickel. The problem which has not hitherto been satisfactorily solved is to put this powder on nickel lead wires and keep it there so distributed that it can effectively act on all three elements, namely hydrogen, oxygen and carbon without adding any more harmful materials.

Other binders and suspending mediums in addition to those mentioned above have been proposed as, for example, silicates, like sodium silicate, but all such binders with which I am familiar add water to the getter which may be almost as detrimental as carbon. Certain phosphates have been proposed as binders but they either add water or phosphoric acid which is also undesirable in lamp making.

Moreover, none of the prior binders proposed or used with which I am familiar acts also as a getter in addition to the binding function.

I have found that potassium fluozirconate ( $K_2ZrF_6$ ) has ideal characteristics for a binder and in addition acts as a getter. The material is a fine white powder which does not absorb water. When mixed with alcohols, acetates, lactates and other solvents this material forms an emulsion which helps to hold the metal powders in suspension. The mixture makes a nice painting or spraying medium applied as a thin continuous film. As the liquids evaporate this material forms crystals that hold the metal powders to the nickel leads. As the lamps are processed and heat is applied during the sealing and exhaust operations no further action apparently takes place. When the filaments are burned the extra heat changes the salt from white to dark grey. After this change the getter is porous but is fastened to the nickel wire very tightly requiring decided force to break it loose. The extra heat probably breaks the double fluoride apart, the potassium fluoride forming large porous crystals which hold the metal powder in place but will not break down until a temperature of  $1200^{\circ} C.$  or above is reached. The zirconium fluoride is probably a gas at  $500^{\circ} C.$ , the temperature which the lamp leads ordinarily reach while burning. This either recrystallizes at a lower temperature or breaks up, releasing metallic zirconium and fluorine gas which are both active getters. While this is probably the correct theory of the functioning of the binder and the paint it is understood that the functioning may vary from the theory above expressed.

Any suitable method of forming the getter paint may be employed. The following is a suitable method of making a getter paint embodying potassium fluozirconate as the binder which may be applied by painting the same on the structure with a brush. To 300 grams of potassium fluozirconate, 180 cc. of propanol and 120 cc. of ethyl lactate are added. This mixture is then thoroughly mixed and treated by treating and mixing the same in a small ball mill for a suitable period. This period may be for six-

3-

teen hours or less. To this mix is added around 1200 grams zirconium powder, dampened with propanol and ethyl lactate as, for example, around 480 cc. propanol and 320 cc. ethyl lactate. The whole is thoroughly mixed in any suitable manner. The paint is then ready for application by brush. It may be conveniently stored for use in bottles as, for example, bottles of 100 cc. capacity.

If instead of applying the paint by brush it is desired to spray it on the lamp structures or parts involved, a different set of thinners is desirable or necessary to increase the drying speed. For example, a good spray mixture could be made by taking 100 cc. of the brush on mix and adding 100 cc. of butyl acetate, 150 cc. of ethyl alcohol, and 50 cc. of ether.

Another mixture that would be good could be made up using 1 part ethyl lactate, 3 parts amy1 acetate, and 4 parts methanol. The solids should be thinned down to about the same specific gravity as the above mixture.

Special precautions must be observed in the use or handling of metallic zirconium as, for example, all water must be removed without drying the powder. This may be done by decanting with either methanol or propanol. In addition, if 10% aluminum silicate or other inert material is added to the zirconium the whole batch may be milled together safely, thus making a smoother mix.

I claim:

1. A getter paint comprising about 1200 parts by weight of metallic zirconium powder dampened with propanol and ethyl lactate and ther-

oughly admixed with 300 parts by weight of potassium fluorzirconate, in about 180 parts by volume of propanol and 120 parts by volume of ethyl lactate.

5 2. A getter paint comprising powdered metallic zirconium thoroughly admixed with potassium fluozirconate as a binder and dispersed in a sufficient amount of a volatile organic solvent vehicle to form a non-viscous liquid for coating  
10 smooth metal surfaces, the weight of the powdered metal zirconium exceeding the weight of the potassium fluozirconate in the paint.

## LLOYD D. LOCKWOOD.

#### REFERENCES CITED

The following references are of record in the file of this patent:

UNITED STATES PATENTS

|    |           |          |               |
|----|-----------|----------|---------------|
| 20 | Number    | Name     | Date          |
|    | 1,698,850 | Marden   | Jan. 15, 1929 |
|    | 1,895,855 | Lockwood | Jan. 31, 1933 |
|    | 1,958,967 | Kniepen  | May 15, 1934  |
|    | 2,108,617 | Schroter | Feb. 15, 1938 |
| 25 | 2,167,762 | Lockwood | Aug. 1, 1939  |
|    | 2,263,164 | Dailey   | Nov. 18, 1941 |

## FOREIGN PATENTS

| Number  | Country       | Date          |
|---------|---------------|---------------|
| 547 645 | Great Britain | Sept. 4, 1942 |

#### OTHER REFERENCES

Mellor, Comprehensive Treatise on Inorganic and Theoretical Chem., 1927, vol. 7, pages 138 and 140.